

L. P. BURROWS.

## METHOD OF TREATING SILVER ORES.

APPLICATION FILED DEC. 5, 1916. RENEWED NOV. 1, 1919.

1,355,795.

Patented Oct. 12, 1920.



WITNESSES

Wm. A. Gray.

INVENTOR  
L.P.BURROWS.

57 *Leicesterhaugh & Co.* 1911/5.

માનુષ.

# UNITED STATES PATENT OFFICE.

LINUS PORTER BURROWS, OF OTTAWA, ONTARIO, CANADA.

## METHOD OF TREATING SILVER ORES.

1,355,795.

Specification of Letters Patent.

Patented Oct. 12, 1920.

Application filed December 5, 1916, Serial No. 135,223. Renewed November 1, 1919. Serial No. 335,108.

To all whom it may concern:

Be it known that I, LINUS PORTER BURROWS, a citizen of the United States, and residing at 380 McLeod street, in the city of 5 Ottawa, Province of Ontario, Dominion of Canada, professor, have invented certain new and useful Improvements in Methods of Treating Silver Ores, of which the following is a specification.

10 This is a discovery and relates to the recovery of silver and other metals from silver ore and its result is the obtainment of a maximum amount of the metals in purified form in a minimum of time as well as rendering commercially practicable the treatment of ores of such low grade as has heretofore been impossible.

15 The discovery consists in a method of treating the ore directly with the gas described in my Patent No. 680,313, in any suitable apparatus such as the one shown in the accompanying drawings which show a sectional elevation of the apparatus.

20 The apparatus comprises an expansion, a radiation and precipitation chamber A, a digester B and a plurality of precipitating chambers C, only one of which is shown. The digester B includes a treating chamber E, in which the material is treated. For 25 convenience in agitating the material the treating chamber is constructed in the form of a rotatable drum having hollow side trunnions 10 and 11 secured to the ends 12 and 13 of the drum.

30 Suitable means are provided for heating the material in the drum. In the embodiment illustrated I have surrounded the treating chamber with a furnace or heating chamber F constructed with a suitable sheet metal shell 14 lined with firebrick, or other heat resisting material 15. The heating 35 may be accomplished by any well known means such as a gas burner 16 supplied with a gas supply pipe 17.

40 The air for combustion of the gas may pass in through the opening 18, and the products of combustion flow out through the opening 19.

45 The turning of the treating chamber is accomplished by convenient means, such as the gear 20 mounted on the trunnions 11 and driven from the pinion 21 on the countershaft 22, which counter shaft is supported by suitable bearings 23 and 24 and driven

from a pulley 25. The trunnions 10 and 55 11 are supported by bearings 26 and 27.

The expansion, radiation and precipitation chamber A is in the form of a cylindrical metallic container of metal preferably sheet iron, in which the steam is adapted 60 to suddenly expand from substantially the center of the container, being introduced from the center by a pipe 40 which extends through the side of the chamber. On the top of the chamber is a dome 41 from which 65 the crude gas or gases pass into a delivery pipe 42.

A weighted pop valve 43 leads from the pipe 8 into the atmosphere and serves to maintain a substantially uniform pressure 70 in the said pipe. The pipe 42 also contains a control valve 44.

The water of precipitation is removed by a suitable valved outlet 45 at the bottom of the chamber controlled by a ball float 46 which 75 causes the water to flow off as soon as it rises to any considerable height in the bottom of the chamber. A manhole 47 may be provided normally closed by a door 48.

The steam produced from water which 80 forms the base of the gaseous product may be produced in any convenient way. After the process is started it may be produced by the heat radiating from the furnace F, and accordingly a heating coil H is shown embedded in the walls of the furnace supplied by a pipe 51 leading from a suitable source of water supply.

85 From the coil H a pipe 52 leads to the chamber A. From the chamber A the resultant gaseous product passes by the pipe 42 and a pipe 53 to suitable coils I in the chamber F, whereby the gas is heated to a high temperature. From the heating coils I, the resultant gaseous product passes by the 90 pipe 54 to the valved injecting nozzle 55 which projects through the hollow trunnion 10 having a gas tight joint therewith. The gaseous product is discharged through the 95 nozzle F into the chamber E to act upon the substances therein. A suitable pressure gage 56 may be provided to indicate the pressure at this point and the flow may be controlled by a suitable valve 57.

100 The gaseous products of the reaction in the chamber E passes through the hollow conduit 60 leading to the side of the first precipitating chamber C. A plurality of

similar precipitation chambers will be provided connected in series.

The above description of the making of the gas forms no part of this invention as 5 it is only a reiteration of the method disclosed in my Patent No. 680,313.

In practically carrying out the process a suitable quantity of silver ore, such as cobalt silver ore usually an arsenide or sulfide of silver with varying quantities of cobalt nickel, is ground to 40 mesh and placed in the chamber E, which is then continuously rotated and heated to red heat during the operation of the process.

15 The gaseous reagent made in accordance with Patent 680,313 is continuously injected into the ore rotating in the chamber E until the refining is carried to the desired point, the time which this occupies for a given ore 20 being ascertained by test but is only a matter of hours.

The material in the container F is then removed and smelted in a crucible furnace or any other convenient way to separate the 25 metal from the gangue or silicious material, a flux may be used if necessary to facilitate the smelting.

After cooling the crucible, its contents are dumped out and found to be in the form of 30 superposed distinct layers or cakes, silver being on the top of the pile, then the other metals of the ore such as cobalt, nickel, etc., and then the slag which takes a decidedly crystalline form.

35 In carrying out the process in connection with ores having an acid character it may be found desirable to add counteracting substances such as sodium chlorid or potassium chlorid, the same being inserted in the chamber E.

40 As many changes could be made in the

above invention and many apparently widely different embodiments of my invention within the scope of the claims constructed without departing from the spirit 45 or scope thereof, it is intended that all matter contained in the accompanying specification and drawings shall be interpreted as illustrative and not in a limiting sense.

I claim—

1. A method of the class described consisting in first suddenly expanding steam, then separating the steam without condensation from any water held in suspension, then heating the gaseous product to a high 55 temperature, and subjecting crushed silver ore to the gaseous product at red heat, smelting the treated ore, and cooling the result whereupon the different metals contained in the ore are found to be in purified 60 condition and in separate layers.

2. The method of claim 1 in which a chlorid of an alkaline earth metal is added to the ore before treatment with the gas.

3. The herein described process consisting in first suddenly expanding steam, then separating the steam from any water held in suspension, then heating the gaseous product to a high temperature and subjecting crushed silver ore containing a metal of the iron group to the action of said gaseous product in a closed cylinder at a red heat and thereafter subjecting said treated and refined ore to a smelting process, the resultant product being stratified into magnetic and non-magnetic metal when cold, the resultant silver product being of from 800 to 900 fine.

70 In witness whereof I have hereunto set my hand.

LINUS PORTER BURROWS.